

Patented Sept. 30, 1941

2,257,668

# UNITED STATES PATENT OFFICE

2,257,668

## FORMATION OF PROTECTIVE LAYERS ON IRON AND STEEL ARTICLES

Gottfried Becker, Dusseldorf, and Fritz  
Steinberg, Krefeld, Germany

No Drawing. Application March 12, 1937, Serial  
No. 130,586. In Germany November 10, 1934

1 Claim. (Cl. 91—70.1)

The present invention relates to improvements in or relating to the formation of protective layers on iron or steel articles by forming a layer of chromium or a chromium alloy at or within the surface thereof, the forming of such a layer on the article surface for convenience in terminology herein called "chromising" the surface.

It is an object of the present invention to provide an improved process for forming protective layers on iron and steel articles which can be carried out continuously in a controlled manner.

It is a further object of the invention to provide a method of forming protective layers on articles of iron or ferrous metals such as steel by treating them with gaseous chromous chloride at an elevated temperature.

It is a further object of the invention to provide a method of forming protective layers on articles of iron or ferrous metals such as steel by treating them in a gaseous mixture comprising chromous chloride and hydrogen.

It is a further object of the present invention to provide an improved method of forming protective layers on iron or steel articles by heating them to about 900° C. or over in an atmosphere resulting from the reaction of a mixture of hydrogen and hydrogen chloride on chromium or a chromium alloy especially ferrochrome.

An important feature of the present invention resides in the use of gaseous chromous chloride or the gas atmosphere above referred to as distinct from chromic chloride as such.

According to the present invention, we provide a method of forming protective layers on iron and steel articles including the steps of passing a mixture of hydrogen and hydrogen chloride over heated chromium or chromium alloys and causing or allowing the resultant gaseous product to act on the articles at a temperature of about 900° C. or over.

The terms "gas or gaseous" as used herein refer not only to true gases but also to vapours.

It is preferred to employ the hydrogen in a large proportion as compared with the quantity of hydrochloric acid. As a result of tests it is believed that the gaseous product contains chromium in the form of chromous chloride and indeed it has been found by extensive research that the formation of the chromium or chromium containing layer proceeds considerably more rapidly and more uniformly than is the case where chromic chloride is employed as such. Moreover in the method of the present invention the chromium containing gas or vapour can be produced continuously and brought to reaction in

5 regulatable amounts or concentration. Moreover the chromium or chromium containing layer may be made of any desired thickness by controlling the reaction conditions or time of treatment.

10 It is indeed surprising that the gaseous or vapourous chromium compound which is believed to be chromous chloride is produced at all under the strongly reducing conditions because it is known that chromium compounds are reduced to metallic chromium when heated in the presence of hydrogen. When a chromium alloy, such for example as ferrochrome is employed it is probable that the hydrogen chloride first attacks the 15 surface of the ferrochrome forming volatile ferrous chloride which of course has no action on the articles to be treated. As the iron is removed from the surface of the ferrochrome leaving chromium, the latter is then attacked by the 20 hydrogen chloride in the presence of hydrogen to form a volatile chromium compound, probably chromous chloride, which as stated above, reacts particularly favourably with the iron or steel. The resulting gas mixture may be passed continuously over the articles to be treated at a 25 regulatable rate whereby the desired exchange of chromium and iron is effected. The chromium penetrates or diffuses into the surface of the articles without substantially altering the dimensions of the original articles. At a temperature of 980° C. and a treating period of 4 to 6 hours a chromium containing layer of a thickness of 30 about 0.1 mm. has been obtained. The articles treated had a smooth lustrous surface and the 35 chromium content of the protective layer was about 25%.

40 The hydrogen and the hydrogen chloride can be produced or supplied from separate sources and mixed with one another or the mixture of hydrogen chloride and hydrogen may be conveniently produced by passing hydrogen at a regulated rate through fuming hydrochloric acid.

45 Either or both of the gases hydrogen chloride and hydrogen or the mixture of the two, may be passed through one or more suitable drying means for example bubbled through concentrated sulphuric acid or passed through drying tubes or towers. This is especially advantageous when producing the mixture of the two gases by bubbling hydrogen through fuming hydrochloric acid.

50 One of the advantages of the method according to the present invention is that by varying the composition of the gas mixture, i. e. the concentration of chromium compound, for example

by varying the initial proportions of hydrogen to hydrogen chloride, or varying the total quantity of gas or varying the reaction temperature or the period of reaction, or varying any desired number of these factors the thickness of the protective layer produced can be varied. Moreover the process can be interrupted at any desired instant.

If desired the articles to be treated, may first be subjected to the action of hydrogen alone whilst being heated for the purpose of removing surface impurities such as oxides. It is therefore generally not necessary to clean the articles before introducing them into the reaction chamber as has previously been considered necessary.

The method of the present invention may be carried out in various ways. The volatile chromium compound can be produced in the same vessel as the article or articles to be treated or in different vessels. Thus for example chromium or an alloy thereof for instance ferrochrome may be placed in one or more retorts or drums and heated to red heat whilst a mixture of hydrogen chloride and hydrogen is passed over it. The gaseous product which is probably a mixture of chromous chloride and hydrogen may then be passed through a drum or other suitable vessel containing the article or articles to be treated, heated to a temperature of about 900° C. or over. It may be of advantage to rotate the drum or other vessel in which the article or articles is/are treated.

In another method of carrying out the invention the mixture of hydrogen chloride and hydrogen is caused to act on the chromium or chromium alloy preferably ferrochrome in the same

chamber or vessel as that in which the article or articles to be treated are placed, but the arrangement should be such that the stream of hydrogen and hydrogen chloride meets the chromium or chromium alloy before reaching the articles to be treated. In this case the chromium or chromium alloy and/or the article or articles to be treated, may be enclosed in suitable perforated or cage like containers. If desired the article or articles to be treated may be placed in a rotary perforated or cage like container arranged within a larger container in which the chromium or ferrochrome is placed. Alternatively a rotary container may contain both the article or articles to be treated and the chromium or chromium alloy, these being separated if desired by a perforated or grid or sievelike partition.

We claim:

A method of chromising the surface portions of iron and steel articles comprising passing a gaseous mixture consisting essentially of hydrogen and chromous chloride from a source of supply through a heated chamber containing the articles so as to cause a stream of said mixture to pass continuously over the articles in contact therewith, whereby said surfaces will be continuously acted upon by a mixture of hydrogen and chromous chloride for a chromising treatment of any duration, the chamber being heated to such temperature as will maintain the articles at at least 900° C., and regulating the rate and duration of flow of said mixture for controlling the thickness of the protective layers.

GOTTFRIED BECKER.  
FRITZ STEINBERG.